# EUROPEAN PATENT SPECIFICATION

(11) **EP 1 350 867 B1**
(45) Date of publication and mention of the grant of the patent: **05.07.2006**
(21) Application number: 03007463.7
(22) Date of filing: 04.04.2003
(51) Int. Cl.: C23C 22/23, C10M 173/02

(54) **A coating solution for metals and metal alloys**
Beschichtungslösung für Metalle und Metallegierungen
Solution de revêtement pour métaux et des alliages de métaux

(30) Priority: 04.04.2002 EP 02007662
(43) Date of publication of application: 08.10.2003
(73) Proprietor: Zepf, Walter, 78467 Konstanz/Bodensee (DE)
(72) Inventor: Zepf, Walter, 78467 Konstanz/Bodensee (DE)
(74) Representative: Müller-Boré & Partner Patentanwälte

(56) References cited:
- EP-A- 0 613 939
- EP-A- 0 714 975
- FR-A- 2 378 084
- US-B1- 6 309 477
- DATABASE CA [Online] CHEMICAL ABSTRACTS SERVICE, COLUMBUS, OHIO, US; IZAKI, TERUAKI ET AL: "Plated steel sheet covered with organic film for high corrosion resistance" retrieved from STN Database accession no. 135:347629 CA XP002213347 & JP 2001 303262 A (NIPPON STEEL CORP., JAPAN) 31 October 2001 (2001-10-31)

## Description

The present invention relates to a coating solution to be applied onto the surface of metals or metal alloys, a process for cold forming of metals and metal alloys using said coating solution, and a coated blank made of a metal or a metal alloy.

In cold forming, no heat is applied to the metallic workpiece before forming. However, its temperature can increase during the forming process, as the energy expanded in forming is almost completely converted into heat. The main advantages of cold forming are the saving of materials and working time, the use of lower strength steels, the improved quality of workpieces, lower machine costs, better size accuracy, high surface quality and an extended tool life. In order to achieve these advantages, a protective film must be formed between the tool and the work piece, which must remain intact during the working process. Such a protective film is mainly made up of molybdenum disulfide dispersions or graphite as lubricants. Hitherto, in order to obtain such a protective lubricating film in cold forming processes, lubricant carriers are applied onto the surface of the workpiece, which can absorb about five times the quantity of lubricants compared to the untreated metal surface. However, the application of such lubricant carriers onto the surface of workpieces is carried out by applying aggressive acids and metallic soaps in huge amounts, which is not desirable from an ecological standpoint.

US-patent 6,309,477 describes pretreatment chemicals for metal materials to be painted containing at least one kind of sulfur-containing compounds and at least one of phosphorus ion-containing compounds, and an anticorrosive treatment of metal materials. JP-A-2001-303262 describes a plated steel sheet covered with an organic film for high corrosion resistance. EP-A-0 613 939 describes a graphite-free lubricating oil which comprises a base oil having dispersed therein a carbohydrate and/or a derivative thereof, a film-boosting agent and a dispersant.

Therefore, the technical problem underlying the present invention is to provide a new system for cold forming of metals and metal alloys, which should avoid the treatment of the working piece with aggressive acids and/or metallic soaps prior to the cold forming process, but should exhibit at least the same results compared to a cold forming process using workpieces treated with aggressive acids and/or metallic soaps.

The solution to the above technical problem is achieved by providing the embodiments characterized in the claims.

In particular, there is provided a coating solution to be applied onto the surface of a metal or a metal alloy, comprising 2 to 8% (w/v) of a polyphosphate, 2 to 5 % (w/v) of a dithiocarbamate, 5 to 12% (w/v) of graphite and 5 to 12 % (w/v) of molybdenum disulfide.

In a preferred embodiment of the present invention, the polyphosphate is selected from the group consisting of ammonium polyphosphate and alkali metal polyphosphates, such as sodium polyphosphate, or mixtures thereof.

The dithiocarbamate is preferably a dialkyl dithiocarbamate, wherein the alkyl groups are the same or different and can have 1 to 12 carbon atoms. In a preferred embodiment of the present invention the dithiocarbamate is a heavy metal dithiocarbamate, wherein the heavy metal is for example molybdenum. In a more preferred embodiment of the present invention the dithiocarbamate is a molybdenum dibutyldithiocarbamate.

In a preferred embodiment of the present invention the coating solution may further contain at least one component selected from the group consisting of alcohols in an amount of from 0 % to about 100% (v/v); waxes such as polyalkylene waxes, e.g. polyethylene waxes, microcrystalline waxes, and Montan ester waxes, in an amount of from 0 % to about 80 (v/v); emulsifying agents such as alkyloxyethylates and alkylaryloxyethylates, in an amount of from 0 % to about 50% (v/v); pH-modulating agents such as buffers, e.g. phosphorous acid and esters thereof, in an amount of from 0 % to about 50% (v/v); polymeric compounds such as polyethylene glycols, preferably having a weight average molecular weight of from 500 to 1,000,000, polysaccharides and methylcellulose, in an amount of from 0% to about 50% (v/v); oxides such as silicon dioxide, in an amount of from 0% to about 50% (v/v); friction-reducing agents such as sodium stearate, in an amount of from 0% to about 80% (v/v); defoaming agents such as fatty alcohol polyglycol ethers, in an amount of from 0% to about 50% (v/v); carboxylic acids and derivatives thereof such as 2-phosphonobutanetricarboxylic acid, in an amount of from 0% to about 50% (v/v); organophosphorous compounds such as alkylphosphates, in an amount of from 0% to about 5% (v/v); and phosphates such as boron phosphate, sodium phosphate, P₂O₅ etc., in an amount of from 0% to about 80% (v/v); and mixtures thereof containing two or more of said components.

In a preferred embodiment of the present invention, the coating solution has a pH-value ranging from about 3 to about 4, adjusted by the above-defined pH-modulating agent.

The solvent used for the coating solution of the present invention is H₂O in an amount of from 0% to 100% (v/v), alcohols, preferably alcohols having up to 10 carbon atoms such as methanol, ethanol, etc., or a mixture of different alcohols, in an amount of from 0% to 100% (v/v), or a H₂O/alcohol-mixture in an amount of from 0% to 100% (v/v).

Further, the present invention relates to a process for cold forming of metals or metal alloys, comprising the steps of:
(a) immersing a blank of a metal or a metal alloy in a bath containing the above-defined coating solution for a time period of from about 30 seconds to about 10 minutes;
(b) drying said blank having the coating solution on its surface at a temperature ranging from about room temperature to about 80°C, preferably from about 50°C to about 60°C, wherein the drying is carried out preferably in hot air or in a drying stove; and
(c) subjecting the thus-coated blank to cold forming.

In the preferred embodiment, the blank can be sand-blasted prior to the above process step (a).

Further, there is provided a blank made of a metal or a metal alloy such as steel, having a coating obtainable by the above-defined process steps (a) and (b).

When using the above-defined coating solution for the treatment of blanks ("workpieces") to be processed in cold forming, there can be observed that on the one hand the coating solution of the present invention does not exhibit the severe drawbacks with respect to environmental pollution, and on the other hand the blanks having a coating based on the coating solution of the present invention show at least the same results for the processed workpiece and the tool when compared with blanks having a coating known in the prior art. Moreover, the cold forming process using blanks treated with the coating solution of the present invention is superior from an economical standpoint, i.e. the weight of the coating on the blank is much less as compared to the weight of a coating known in the art. Additionally, in comparison with a coating procedure known in the art, wherein about eleven steps for applying the coating on the blank are necessary, only two steps - (i) immersing the blank in the coating soluting according to the pursuant invention and then (ii) drying the blank - are necessary resulting in a drastically saving of time.

The present invention will now be further illustrated in the following examples, without being limited thereto.

### Examples

25 cylindrically shaped steel blanks (examples 1 to 25) having a length of 500 mm are immersed in a coating solution containing 2-8 % (w/v) polyphosphate, 2-5 % (w/v) dithiocarbamate, 5-12 % (w/v) graphite and 5-12 % (w/v) molybdenum disulfid for a time period of about 1 min. Then, the blanks having the coating solution on their surfaces are transferred to a drying stove wherein they are dried at a temperature of about 60°C for about 30 min. For comparison, 5 cylindrically shaped steel blanks (Comp. Examples 1 to 5) having a length of 500 mm are coated using the agents and procedure known in the art. The results are summarised in Table 1.

**Table 1**

| Examples | blank weight before coating [g] | blank weight after coating [g] | weight of coating [g] | cold forming of coated blanks |
|---|---|---|---|---|
| 1 | 5583.2 | 5584.3 | 1.1 | + |
| 2 | 5558.1 | 5559.6 | 1.5 | + |
| 3 | 5560.3 | 5561.2 | 0.9 | + |
| 4 | 5562.1 | 5563.0 | 0.9 | + |
| 5 | 5552.7 | 5553.9 | 1.2 | + |
| 6 | 5532.6 | 5533.6 | 1.0 | + |
| 7 | 5538.4 | 5539.3 | 0.9 | + |
| 8 | 5552.9 | 5554.8 | 1.9 | + |
| 9 | 5564.1 | 5565.1 | 1.0 | + |
| 10 | 5554.2 | 5555.9 | 1.7 | + |
| 11 | 5553.9 | 5558.7 | 2.8 | + |
| 12 | 5547.6 | 5556.6 | 1.0 | + |
| 13 | 5560.0 | 5561.1 | 1.1 | + |
| 14 | 5568.7 | 5569.6 | 0.9 | + |
| 15 | 5573.0 | 5571.2 | 0.9 | + |
| 16 | 5563.0 | 5563.8 | 0.8 | + |
| 17 | 5572.0 | 5573.0 | 1.0 | + |
| 18 | 5570.6 | 5571.5 | 0.9 | + |
| 19 | 5562.1 | 5563.0 | 0.9 | + |
| 20 | 5559.1 | 5559.9 | 0.8 | + |
| 21 | 5570.7 | 5571.8 | 1.1 | + |
| 22 | 5572.8 | 5573.4 | 0.6 | + |
| 23 | 5561.1 | 5562.7 | 1.6 | + |
| 24 | 5563.2 | 5564.0 | 0.8 | + |
| 25 | 5563.7 | 5564.8 | 1.1 | + |
| Comp. Example | | | | |
| 1 | 5531.0 | 5560.1 | 29.1 | + |
| 2 | 5526.8 | 5557.0 | 30.2 | + |
| 3 | 5535.4 | 5562.3 | 26.9 | + |
| 4 | 5533.4 | 5563.1 | 29.7 | + |
| 5 | 5532.6 | 5551.5 | 18.9 | + |

As can be taken from Table 1, the coated blanks according to the present invention exhibit a drastically reduced coating weight, but the coating reveals at least the same properties for the blank to be cold formed as the coating of blanks obtained according to the prior art, upon evalution of the processed coated blanks during and after their cold forming (+=good results of the formed blanks after 3 operations in a cold forming process).

## Claims

1. A coating solution to be applied on the surface of metals or metal alloys, comprising 2 to 8 % (w/v) of a polyphosphate, 2 to 5 % (w/v) of a dithiocarbamate, 5 to 12 % (w/v) of graphite and 5 to 12 % (w/v) of molybdenum disulfide.

2. The coating solution according to claim 1, wherein said polyphosphate is selected from the group consisting of ammonium polyphosphate and alkali metal polyphosphates, or a mixture thereof.

3. The coating solution according to claim 1 or 2, wherein said dithiocarbamate is a dialkyl dithiocarbamate.

4. The coating solution according to claim 3, wherein said dithiocarbamate is a heavy metal dithiocarbamate.

5. The coating solution according to any one of claims 1 to 4, further comprising at least one component selected from the group consisting of alcohols, waxes, emulsifying agents, pH-modulating agents, polymeric compounds, oxides, friction-reducing agents, defoaming agents, carboxylic acids and derivatives thereof, organophosphorous compounds, and phosphates, or mixtures thereof containing two or more of said components.

6. The coating solution according to any one of claims 1 to 5, having a pH-value ranging from about 3 to about 4.

7. A process for cold forming of metals or metal alloys, comprising the steps of:
(a) immersing a blank of a metal or a metal alloy in a bath containing the coating solution according to any one of claims 1 to 6, for a time period of from about 30 seconds to about 10 minutes;
(b) drying said blank having the coating solution on its surface at a temperature ranging from about room temperature to about 80°C; and
(c) subjecting the thus-coated blank to cold forming.

8. The process according to claim 7, wherein prior to step (a) the blank is sand-blasted.

9. A blank having a coating obtainable by
(a) immersing a blank of a metal or a metal alloy in a bath containing the coating solution according to any one of claims 1 to 6, for a time period of from about 30 seconds to about 10 minutes; and
(b) drying said blank having the coating solution on its surface at a temperature ranging from about room temperature to about 80°C, resulting in a coated blank.

## Patentansprüche

1. Beschichtungslösung, die auf die Oberfläche von Metallen oder Metalllegierungen aufzubringen ist, umfassend 2 bis 8 % (Gewicht/Volumen) eines Polyphosphats, 2 bis 5 % (Gewicht/Volumen) eines Dithiocarbamats, 5 bis 12 % (Gewicht/Voiumen) Graphit und 5 bis 12 % (Gewicht/Voiumen) Molybdändisulfid.

2. Beschichtungslösung nach Anspruch 1, wobei das Polyphosphat aus der Gruppe, bestehend aus Ammoniumpolyphosphat und Alkalimetallpolyphosphaten, oder einem Gemisch davon, ausgewählt ist.

3. Beschichtungslösung nach Anspruch 1 oder 2, wobei das Dithiocarbamat ein Dialkyldithiocarbamat ist.

4. Beschichtungslösung nach Anspruch 3, wobei das Dithiocarbamat ein Schwermetalldithiocarbamat ist.

5. Beschichtungslösung nach einem der Ansprüche 1 bis 4, welche ferner mindestens eine Komponente, ausgewählt aus der Gruppe, bestehend aus Alkoholen, Wachsen, Emulgatoren, pH-modulierenden Mitteln, Polymerverbindungen, Oxiden, reibungsverringernden Mitteln, Entschäumungsmitteln, Carbonsäuren und Derviaten davon, Organophosphorverbindungen und Phosphaten, oder Gemische davon, welche zwei oder mehrere der Komponenten enthalten, umfasst.

6. Beschichtungslösung nach einem der Ansprüche 1 bis 5, welche einen pH-Wert in einem Bereich von etwa 3 bis etwa 4 aufweist.

7. Verfahren zum Kaltformen von Metallen oder Metalllegierungen, umfassend die Schritte:
(a) Eintauchen eines Rohlings eines Metalls oder einer Metalllegierung in ein Bad, welches die Beschichtungslösung nach einem der Ansprüche 1 bis 6 enthält, für eine Zeitdauer von etwa 30 Sekunden bis etwa 10 Minuten,
(b) Trocknen des Rohlings mit der Beschichtungslösung an dessen Oberfläche bei einer Temperatur in einem Bereich von etwa Raumtemperatur bis etwa 80°C und
(c) Unterziehen des derart beschichteten Rohlings einem Kältformen.

8. Verfahren nach Anspruch 7, wobei der Rohling vor Schritt (a) sandgestrahlt wird.

9. Rohling mit einer Beschichtung, erhältlich durch
(a) Eintauchen eines Rohlings eines Metalls oder einer Metalllegierung in ein Bad, welches die Beschichtungslösung nach einem der Ansprüche 1 bis 6 enthält, für eine Zeitdauer von etwa 30 Sekunden bis etwa 10 Minuten und
(b) Trocknen des Rohlings mit der Beschichtungslösung an dessen Oberfläche bei einer Temperatur in einem Bereich von etwa Raumtemperatur bis etwa 80°C,
was zu einem beschichteten Rohling führt.

## Revendications

1. Solution de revêtement à appliquer sur la surface de métaux ou d'alliages de métaux, comprenant 2 à 8 % (p/v) d'un polyphosphate, 2 à 5 % (p/v) d'un dithiocarbamate, 5 à 12 % (p/v) de graphite et 5 à 12 % (p/v) de disulfure de molybdène.

2. Solution de revêtement selon la revendication 1, dans laquelle ledit polyphosphate est choisi dans le groupe constitué par le polyphosphate d'ammonium et les polyphosphates de métaux alcalins, ou un mélange de ceux-ci.

3. Solution de revêtement selon la revendication 1 ou 2, dans laquelle ledit dithiocarbamate est un dithiocarbamate de dialkyle.

4. Solution de revêtement selon la revendication 3, dans laquelle le dithiocarbamate est un dithiocarbamate de métal lourd.

5. Solution de revêtement selon l'une quelconque des revendications 1 à 4, comprenant en outre au moins un composant choisi dans le groupe constitué par les alcools, les cires, les agents émulsifiants, les agents modulant le pH, les composés polymères, les oxydes, les agents réduisant le frottement, les agents anti-mousse, les acides carboxyliques et les dérivés de ceux-ci, les composés organophosphoreux et les phosphates, ou les mélanges de ceux-ci contenant deux ou plus desdits composants.

6. Solution de revêtement selon l'une quelconque des revendications 1 à 5, ayant une valeur de pH allant d'environ 3 à environ 4.

7. Procédé pour former à froid des métaux ou des alliages de métaux, comprenant les étapes consistant à :
(a) immerger un flan d'un métal ou d'un alliage de métal dans un bain contenant la solution de revêtement selon l'une quelconque des revendications 1 à 6, pendant une période allant d'environ 30 secondes à environ 10 minutes ;
(b) sécher ledit flan ayant la solution de revêtement sur sa surface à une température allant d'environ la température ambiante à environ 80 °C ; et
(c) soumettre le flan ainsi revêtu à une formation à froid.

8. Procédé selon la revendication 7, dans lequel avant l'étape (a) le flan est décapé au sable.

9. Flan ayant un revêtement pouvant être obtenu par les étapes consistant à
(a) immerger un flan d'un métal ou d'un alliage de métal dans un bain contenant la solution de revêtement selon l'une quelconque des revendications 1 à 6, pendant une période allant d'environ 30 secondes à environ 10 minutes ; et
(b) sécher ledit flan ayant la solution de revêtement sur sa surface à une température allant d'environ la température ambiante à environ 80 °C, conduisant à un flan revêtu.
